

July 24, 1956

G. F. BARNETT

2 756,167

METHOD OF MANUFACTURING CATHODE-RAY TUBE SCREEN STRUCTURES

Filed July 10, 1953

FIG. 2.



FIG. 3.



FIG. 1.

INVENTOR.  
GUY F. BARNETT  
BY  
Oscar U. Hayne  
ATTORNEY

1

2,756,167

## METHOD OF MANUFACTURING CATHODE-RAY TUBE SCREEN STRUCTURES

Guy F. Barnett, Roslyn, Pa., assignor to Philco Corporation, Philadelphia, Pa., a corporation of Pennsylvania

Application July 10, 1953, Serial No. 367,181

14 Claims. (Cl. 117—217)

The invention relates to an improved method of manufacturing cathode ray tube screen structures and also to an improved composition for use in the practice of the method. In particular, the invention relates to an improved method of depositing certain layers of a multi-layer screen structure.

While not limited thereto, the invention is particularly applicable to the manufacture of screen structures for cathode ray tubes for use in reproducing color television images. Accordingly, the invention will be described in detail with reference to its use in color television reproduction.

In certain presently proposed systems of color television, there is transmitted and subsequently received a signal which is representative, at time-spaced intervals, of intelligence concerning the different primary color components of successively scanned portions of a televised scene. It has been recognized that an image of this scene can be reproduced if the received signal is applied to a cathode ray tube and is there utilized to control the intensity of the electron beam at the same time that the beam is deflected across screen elements, each one of which is emissive of light of one of the aforementioned different primary colors. In such a receiver system it is of paramount importance to insure coincidence between the intervals during which the beam intensity is representative of intelligence concerning a particular color and the intervals during which the beam is impinging upon a screen element emissive of light of that same primary color. A scheme which has proven successful in maintaining such coincidence involves the production of electrical signals indicative of beam impingement upon certain screen portions, called "indexing" elements, which are located in known geometrical relation to the light emissive screen elements. These same signals are then utilized to control either the rate of scan of the beam across the screen elements, or the rate of application of intelligence representative signal portions to the beam intensity control grid of the cathode ray tube, or both.

It has been recognized that a particularly advantageous form which such a screen structure may take comprises a substrate made of a transparent dielectric material, such as glass, upon whose electron beam confronting side are deposited the phosphors which constitute the light emissive screen elements. These elements are preferably in the form of narrow, closely spaced parallel strips of phosphor materials, adjoining strips being emissive of light of different primary colors, but any other geometrical configuration may be used for these screen elements which is appropriate to the pattern traced by the electron beam upon the screen structure and to the order of occurrence of color representative portions of the received signal. Upon the beam confronting side of these phosphor elements there is next deposited a thin film of electron permeable conductive material and on this conductive film there is deposited, in turn, a plurality of the aforementioned indexing elements in known geometrical relation-

2

ship to the pattern of the phosphor elements beneath the conductive film. These indexing elements are characterized in that they are made of a material which responds differently to beam impingement than do those portions of the conductive film on which no indexing elements are deposited. If, as is often the case, the conductive film is made of aluminum, which is known to have a comparatively low secondary electron emission ratio, then the indexing elements may appropriately be made of a material having a substantially higher secondary electron emission ratio than aluminum. If there is further provided a suitably energized collector electrode for secondary electrons emitted from the screen structure in response to beam impingement, then a much larger number of secondary electrons will flow from the screen to the collector electrode during intervals when the electron beam impinges upon indexing elements than during intervals when the beam impinges upon portions of the aluminum layer which are not covered with indexing elements. These variations in intensity of secondary electron flow produce corresponding variations in the current flow through an external circuit connecting the collector electrode to the aluminum film. The latter current variations constitute the aforementioned indexing signals and can be utilized in any conventional manner. A screen structure of the type generally described hereinbefore, and associated circuitry for utilizing the indexing signals which it produces to assure beam impingement registry, is disclosed in the copending U. S. patent application of Carlo V. Boccia-  
relli, Serial No. 198,709, filed December 1, 1950, and assigned to the assignee of the present invention.  
Alternatively the indexing elements may be formed of light emissive phosphor materials. In that event, impingement of the beam upon an indexing element will cause the emission of light from this element toward the interior of the tube, while impingement of the electron beam upon portions of the aluminum layer on which no indexing elements are deposited will produce no light emission toward the interior of the tube. Consequently a photoelectric cell, which views the screen structure from the interior of the cathode ray tube, will be subjected to variations in intensity of illumination as the electron beam traverses alternately indexing elements and bare aluminum portions between indexing elements. In response to these light variations the photoelectric cell will generate a varying output current which may again be utilized as the indexing signal. It will be noted that, in any case, light is also emitted from the image producing phosphors in response to electron beam impingement. However, this light emission takes place on the side of the aluminum film which faces away from the photoelectric cell and will be prevented from affecting the photocell by the aluminum film which is not transmissive of such light to any substantial degree.  
In fact, it will now be recognized that the aluminum film acts to separate from each other, both optically and electrically, materials which are deposited on opposite sides thereof, for not only is light incapable of penetrating this film but so are secondary electrons. Consequently, where secondary electrons are used for indexing, those which are emitted from the phosphor elements of the screen structure in response to beam impingement will be intercepted by the aluminum film before they can contaminate the indexing indications produced by secondary electrons emitted from the indexing elements. When light is used for indexing, the aluminum film prevents light from the image productive phosphors from contaminating the indexing indications. This isolation, both electrical and optical, of the materials deposited on opposite sides of the aluminum layer makes the use of such an aluminum film especially desirable for indexing purposes. Of course

it will be understood that, in its application to a color television cathode ray tube, the aluminum film retains the light intensifying property for which its presence has long been valued in black-and-white television picture tubes.

While the desirability of the foregoing type of screen structure has been recognized, it has not been widely adopted because serious difficulties are encountered when its manufacture is attempted. While all of the steps involved in the manufacture of such a screen structure are comparatively difficult, none is more forbidding than the step of forming the indexing elements on top of the aluminum film. The reason for this will be readily understood when it is recalled that the aluminum layer must be extremely thin in order to permit the electron beam to traverse it without prohibitive attenuation. As a matter of fact, it is well known from experience with black-and-white picture tubes that the thickness of the aluminum film must be limited to about 1000 Angstrom units, or 4 millionths of an inch. The deposition of a comparatively heavy layer of indexing material on such a tenuous film would obvious be a touchy operation even if the aluminum film itself were firmly supported. In practice, however, no such firm support exists. This is because the light emissive screen on which the aluminum film is formed consists of aggregates of discrete phosphor particles, many of which protrude irregularly from the film confronting surface of the screen. The aluminum film, which must be optically smooth if its potentialities for intensifying the televised image are to be realized, must therefore be stretched, unsupported, across the gaps between these protrusions. It is to be expected that, in its unsupported regions, a metallic film as thin as the aluminum film in question will have very little mechanical strength. This expectation was confirmed as soon as it was attempted to deposit the additional material required for formation of the indexing elements on top of this aluminum film by any of the orthodox methods which have been used in the past for the deposition of various screen materials. If the particles additionally deposited were comparatively large, then their mass was also relatively great and they would rupture the tenuous aluminum film at the points where they contacted it. This occurred even though special precautions were taken to deposit the particles as gently as possible. If, on the other hand, the particle size was decreased to the point where damage from impact became less likely, then the particles tended to penetrate the aluminum film through minute, intermolecular apertures therein and to produce swelling of the organic gel on which the aluminum film is supported during screen structure formation, again causing rupture and blistering of the aluminum. In fact it has been found that, of any given number of screens which were successfully aluminized, only a very small percentage had a fault-free aluminum film after application of the indexing material. This difficulty was particularly troublesome because the faulty portions of the aluminum film were often hidden beneath the indexing elements and were therefore discoverable only after the tube had been completed and had been tested under actual operating conditions. When a fault was discovered at this late stage of the manufacturing process, the entire tube had to be scrapped. As might be expected, the combination of the foregoing difficulties increased the unit cost of each successfully produced tube to the point where the entire operation became commercially impractical. The problem was further aggravated by the continuing trend toward tubes with ever larger screens, as it was found that the percentage of tubes with satisfactory aluminum films decreased appreciably each time the size of the screen was increased.

Accordingly it is a primary object of the invention to provide an improved method of manufacturing cathode ray tubes.

It is another object of the invention to provide an

improved method of manufacturing cathode ray tube screen structures.

It is still another object of the invention to provide an improved method of manufacturing cathode ray tube screen structures having a light reflective, electron permeable film of conductive material superposed on the image productive phosphors of the screen and having additional material superposed on said film of conductive material.

It is a still further object of the invention to provide an improved method of manufacturing cathode ray tube screen structures suitable for use in color television picture tubes.

Still another object of the invention is to provide an improved method of manufacturing a screen structure for a color television picture tube, the screen structure comprising an array of phosphor elements emissive of light of different primary colors disposed in a predetermined geometrical pattern, an electron permeable aluminum film supported by said phosphor elements, and indexing elements supported by said aluminum film and disposed in known geometrical pattern relative to the pattern of the phosphor elements.

A still further object of the invention is to provide an improved composition for use in my improved method of manufacturing cathode ray tube screen structures.

The foregoing objects of the invention, as well as others which will appear hereinafter, are realized in the following manner. First there is produced, on a suitable substrate by conventional techniques, a phosphor screen of any desired form with a superposed aluminum film or layer for the purposes hereinbefore mentioned. The phosphor screen may be deposited by any of the conventional procedures hereinbefore mentioned, and an organic film or layer may then be applied to the phosphor screen by conventional procedures to condition it for the subsequent application of an aluminum film or layer which likewise is laid down by conventional techniques. As hereinbefore stated, it has not heretofore proved feasible to deposit either secondary emissive or light emissive indexing materials directly on this aluminum layer without grave danger of irreparably damaging either the aluminum layer and/or the underlying phosphor screen. I have discovered, however, that it is feasible to deposit directly on the aluminum layer a layer of suitable organic material which has the effect of protecting the aluminum layer and permitting the subsequent application to it of the desired indexing materials. If desired, after the indexing materials have been so deposited on the reinforced aluminum film, the entire structure may be dried and baked to eliminate the film of organic material so that the indexing elements will then adhere directly to the aluminum film. While in the past, and as hereinbefore mentioned, it has been customary to apply such an organic film to a phosphor screen before the application of an aluminum film, it should be noted that the problems there involved are not the same as those which gave rise to the present invention and it would not have been apparent to one skilled in the art that it would be possible to apply an organic film on an aluminum layer which in turn was superimposed on a phosphor screen. Moreover it would not have been apparent to one skilled in the art that the prior application of such an organic film to the aluminum film would make it possible to apply other materials, such as the indexing materials hereinbefore mentioned, to the surface of the aluminum film. Indeed it could only reasonably be concluded, from the fact that attempts to deposit indexing materials directly on the aluminum film were unsuccessful and resulted in damage to the film and to the underlying phosphor screen, that an attempt to apply an organic film to the aluminum layer would result in similar damage to the aluminum and to the underlying phosphor screen. In fact this was the conclusion reached, prior to the making of the present invention, by numerous experts in the

field who had all but abandoned the hope of applying other materials over such an aluminum film. The reasons for this will be appreciated more fully from a consideration of the differences between the problems presented in the present instance and in the prior art. These will be more readily apparent after my invention has been explained in detail, and accordingly will be discussed more fully hereinafter.

As will be seen from the detailed description of the invention which is to follow, the practice of my invention makes feasible, for the first time, the manufacture of cathode ray tube screen structures of the type under consideration of virtually any desired size with substantial freedom from blemishes in the aluminum film caused by the application of the indexing material.

The particular method of manufacturing cathode ray tube screen structures in accordance with my invention is explained in detail with reference to the accompanying drawings, in which:

Figure 1 is a greatly enlarged fragmentary view of the form of screen structure resulting from the manufacturing process which embodies my invention;

Figure 2 is a flow chart of the steps which characterize the process of my inventive method; and

Figure 3 is a flow chart of an alternative method of manufacturing the screen structures of Figure 1 in accordance with my invention.

The structure of the cathode ray tube screen illustrated in Figure 1 of the drawings, to which more particular reference may now be had, is entirely conventional in all respects, consisting of a glass substrate 10 which may be either the face plate of the cathode ray tube itself or a separate glass plate supported within the tube envelope. Upon this glass substrate there are disposed a plurality of vertical phosphor strips, of which those designated 11 are made of a fluorescent material emissive of red light in response to impingement by the electron beam of the cathode ray tube. Those strips designated 12 are made of a fluorescent material responsive to electron beam impingement to emit green light, while those designated 13 are responsive to emit blue light. As is also conventional, the entire surface area of these strips 11, 12 and 13 is covered by a film 14 of a highly light reflective, conductive material such as aluminum and sufficiently thin to be permeable to the electrons of the cathode ray beam. On the electron beam confronting side of this aluminum film 14 there are in turn disposed a plurality of so-called indexing strips 15, which are arranged in a predetermined geometrical relationship with respect to the phosphor strips 11, 12 and 13 and which are normally characterized by having a secondary electron emission ratio which differs substantially from that of the aluminum film. In practice the indexing strips 15 will frequently be disposed as shown, namely in alignment with phosphor strips emissive of light of one particular color, green for example. There will then be an indexing strip superposed upon every third phosphor strip and separated therefrom by the aluminum film 14. However, it will be understood that this particular arrangement of indexing strips is not essential to my inventive concept. Rather, the particular indexing strip arrangement shown here is purely exemplary and any other configuration of such indexing strips relative to the phosphor screen elements may be obtained by the application of the principles hereinafter set forth. Suitable materials of which these indexing strips may be made include principally those having an electron emission ratio which is considerably higher than that of the aluminum layer. A variety of materials, such as magnesium oxide, barium oxide, strontium oxide, calcium oxide and magnesium orthosilicate have this property.

One particular mode of practicing the method which constitutes my invention is illustrated in the flow diagram of Figure 2, to which more particular reference may now be had. This method starts with the deposition of the

phosphor strips on the glass substrate 10 of Figure 1. This operation is symbolized by rectangle 16 of Figure 2. It may be carried out in a variety of well known ways, as, for example, by settling, silk screening, or photographically depositing the various phosphor strips. In practice I prefer to use the latter method which consists of first applying a uniform coating of one of the fluorescent materials to the entire glass substrate, together with a photosensitive emulsion, then exposing portions of this fluorescent material through transparent slit-like portions in an otherwise opaque mask, these transparent portions having been formed at positions corresponding to the desired locations of strips of that particular phosphor. This exposure fixes the phosphor of the exposed portions and the remaining, unexposed phosphor is washed off. This process is repeated successively with each of the other two phosphors, the mask being relocated each time so as to permit exposure of the proper portions of the phosphor which it is desired to have remain on the glass substrate. The aforescribed process is similar to that described in detail in the copending U. S. patent application of John W. Tiley, Serial No. 248,356, filed September 26, 1951 and assigned to the assignee of the present invention. A variety of phosphors are known which lend themselves to this process of manufacture. Particular phosphors which I have used with success in forming the fluorescent portions of my screen are zinc phosphate for the red light emissive strips, zinc orthosilicate for the green light emissive strips and calcium magnesium silicate for the blue light emissive strips.

The next step in processing the assembly of glass substrate and phosphor strips consists in depositing thereon of an organic film to provide a suitable base for the subsequent deposition of an aluminum film. This step is symbolized by rectangle 17 of Figure 2. Substances are known which are suitable for the formation of such an organic film. For example this film may be constituted of the materials which are disclosed for this purpose in the copending U. S. patent application of Miriam G. Groner, Serial No. 254,195, filed October 31, 1951 and assigned to the assignee of the present invention. The organic film disclosed therein comprises a liquid composition constituted of a small amount of nitrocellulose, a water insoluble plasticizer therefor and octyl acetate dissolved in a mixture of a water soluble alcohol and a volatile ester, the volatile ester being the major constituent of the composition. In particular the alcohol is preferably selected from the group consisting of a propyl alcohol and a butyl alcohol, and the ester is preferably selected from the group consisting of a propyl acetate and a butyl acetate. This liquid composition is permitted to spread over the surface of the previously deposited phosphor strips and also over the exposed portions of the glass substrate wherever, as shown in Figure 1, this glass substrate is not covered by the phosphor strips. This composition is a thin, mobile liquid which readily spreads over the phosphor strips and forms a film containing nitrocellulose, the edges of which adhere to the sides of the cathode ray tube bulb. As is fully explained in the aforementioned Groner application, it is an important advantage of this composition that the alcohols included therein are water soluble and the esters volatile. Because of this, when the composition is applied to the phosphors which, at this stage, contain an appreciable quantity of water left over from the aqueous solution in which they are first deposited, the aforementioned constituents of the film forming composition are gradually removed from the film by being leached out by the aqueous component of the phosphor strips in the case of the alcohol, and by being vaporized into the air above the layer of film forming composition in the case of the volatile esters. This continues until the nitrocellulose containing layer loses its liquid nature and becomes a tacky, flexible, extensible solid film. The octyl acetate, being insoluble in the aqueous material and being of low volatility, remains in the

nitrocellulose film and, along with the plasticizer, imparts thereto the state of tackiness, flexibility and extensibility. When, during the final bake out stage of the completed screen structure, the aqueous suspending medium is completely removed from the phosphor strips, the nitrocellulose film will be caused to sag further and to settle until it rests upon the phosphor strips. The flexibility and extensibility imparted to the film by the octyl acetate in conjunction with the plasticizer permits the film to sag, stretch and otherwise withstand the stresses and distortions involved without breaking. Further drying then removes the octyl acetate and any residual water soluble alcohol and volatile ester from the film, causing the film to shrink and to assume a smooth, stretched character resting on the protruding phosphor particles in the phosphor layer. It will be understood that no invention is predicated on this particular manner of forming the organic film on the phosphor strips, the particular process described being merely illustrative of a preferred mode of accomplishing this step. Other conventional methods of forming this organic film may be used instead, the only requirement being that an organic film be formed whose electron beam confronting surface is sufficiently smooth to permit the deposition of an aluminum film thereon having the desired optical reflecting properties for light which is emitted from the phosphor strips toward the interior of the tube.

The next step of the process, symbolized in Figure 2 by rectangle 18, is the deposition of such an aluminum film. This may be accomplished in any desired manner, as for example by evaporation from a thin aluminum filament suspended near the screen structure and heated to its evaporating temperature by the passage of current directly therethrough, or through a supporting element with which it is in heat exchanging relationship. By control of the evaporation period and of the rate at which evaporation takes place during this period, it is possible readily to control the thickness of this aluminum film. As has been pointed out it is essential that this thickness be limited to such a value that the aluminum film remains electron permeable, for otherwise the electron beam will be unable to excite the colored light emissive phosphors. It is apparent that, the thinner this aluminum film is, the greater will be the fraction of the impinging electron beam which is transmitted to the phosphors and the higher will be the intensity of the light which is emitted by these phosphors in response to a beam of a given intensity. Therefore, even within the limits of electron permeability, it is desirable to make this aluminum film as thin as possible consistently with maintaining its light reflecting properties. As has been indicated it is currently feasible to produce aluminum films which are only about four millionths of an inch thick by the aforementioned evaporation process, by sputtering, or by other conventional methods. Indeed it is the very fact that the use of such extremely thin aluminum films is both necessary and feasible which makes it so difficult to deposit the additional indexing material on the interior surface of the screen structure.

In the formation of the screen structure in accordance with my invention, the next step is symbolically represented by rectangle 19 in Figure 2 and involves the deposition of a second organic film on the exposed surface of the aluminum film formed in step 18. This deposition of an organic film on top of the aluminum film may be carried out in any desired manner, as for example by spraying or by flowing the lacquer onto the aluminum film. In any case, however, care should be taken that as little pressure as possible is applied to the aluminum film during deposition of the organic film thereon. Accordingly, when spraying the organic film onto the aluminum film, I have used pressures which exceed atmospheric pressure by as little as one half pound per square inch. While it is possible to use, for the organic film applied in step 19, the same material as is used for the organic

10

15

20

25

30

35

40

45

50

55

60

65

70

75

film which is applied prior to the deposition of the aluminum film, i. e. in step 17, it is preferred to use, on top of the aluminum film, a composition which includes no water soluble alcohol but instead includes a higher percentage of plasticizer than the organic film material of step 17. The reason for omitting the water soluble alcohol is that generally at this stage there will be no water present which is capable of leaching out this alcohol. The increase in the percentage of plasticizer is prompted by the desire to cause as little stretching as possible of the organic film on top of the aluminum film, as such stretching might cause the aluminum film to lift up from its position in contact with the underlying materials and particularly from its position on the underlying organic film applied in step 17. This lifting is particularly likely to occur along the outer edges of the screen structure. Naturally such lifting is likely to tear and otherwise damage the aluminum film, thereby destroying the usefulness of the screen structure. The use of additional plasticizer material, as hereinbefore suggested, is permissible in the case of the organic film deposited on top of the aluminum film because the indexing strips, which are to be deposited on this organic film, need not have the optical reflecting properties of the phosphor confronting surface of the aluminum film, so that it is not necessary to provide the same smooth substrate therefor as is provided for the aluminum film by the contraction of the organic film with low plasticizer content upon which the aluminum film rests. A preferred composition of the organic material applied in step 19 under discussion consists of 5 grams of nitrocellulose, 5 milliliters of a plasticizer whose chemical name is di-2-ethylbutyrate triethylene glycol and which is sold by the Carbide and Carbon Chemical Company as type 3GH "Flexol," and 250 milliliters of iso amyl acetate.

The next, and penultimate step of the process of Figure 2, symbolically represented therein by rectangle 20, involves the deposition of the indexing strips. This may be carried out in any conventional manner, as, for example, in the same manner as the deposition of the phosphor strips on the glass substrate. In the event that these phosphor strips are deposited by the photographic process hereinbefore outlined, it suffices to deposit the material of which the indexing strips are to be constituted on the organic film formed in step 19 in a suitable photosensitive solution, after which the solution may be exposed to illumination through the same mask which was used for the formation of the phosphor strips, care being taken to reposition this mask so that the transparent portions permit light to fall upon the portions of the screen structure on which indexing strips are to be formed. It should be noted, in this connection, that it is entirely feasible to expose the indexing material which is located on top of the organic film through all of the previously formed portions of the screen structure, and in particular through the aluminum film formed in step 18, provided a sufficiently intense source of illumination is used and provided this exposure is continued for a sufficiently long interval. Alternatively it is possible to expose the materials used in the deposition of the phosphor strips of step 16 from the face plate side of the screen structure and to expose the indexing material from the beam confronting side of the screen structure. However, this latter method involves serious problems of registry between the mask or masks used for the selective exposure from opposite sides and it is preferred to carry out all the exposures from the same side of the screen structure, whether this be the face plate side or the beam confronting side.

The final step of the process, symbolized by rectangle 21 in Figure 2, consists in drying and baking the screen structure formed by the foregoing steps 16 to 20 inclusive. While the drying operation may be carried out at any time, the baking is preferably done after the screen structure has been incorporated into the tube envelope and after

other conventional components of the cathode ray tube have also been placed therein in their usual locations.

It will now be apparent that the organic film, which is deposited on top of the aluminum film, plays an entirely different role in my screen manufacturing method than does the organic film which is deposited beneath the aluminum film. In particular, the organic film beneath the aluminum film is provided for the purpose of forming a smooth surface to which the aluminum film will conform upon deposition, so that the aluminum film will acquire the desired optical reflecting properties. So far as the deposition of the aluminum film itself is concerned, the fragility of the underlying material is clearly no problem, since the glass substrate, as well as the phosphor strips which are formed thereon, are sufficiently sturdy to support not only the weight of the thin aluminum film but also the weight of structures many times as heavy as this film, such as, for example, the indexing strips deposited on the back of the aluminum film. On the other hand, the second organic film, which is deposited on top of the aluminum film prior to application of the indexing strips, is provided for the purpose of insuring that the subsequent application of the indexing material will cause no damage to the extremely fragile aluminum film beneath. That the organic film is capable of affording such protection, without itself damaging the aluminum film, is a fact which previous experience with the use of organic films as the supporting media for the aluminum films had not suggested in any way. On the contrary, prior experience with organic films tended to indicate that comparatively heavy particles, such as those used in the formation of the indexing strips, would readily traverse an organic film and continue to penetrate the aluminum layer beneath, with consequent damage to this aluminum film. As a matter of fact, it was the universal view of those skilled in the art prior to my invention that the thin aluminum film used in cathode ray tube screen structures was quite incapable of supporting any appreciable weight without rupture, so that the application of any substance whatsoever to its beam confronting surface was considered to be impractical.

It is also considered to be noteworthy that the protection against damage resulting from the application of substances to the aluminum film, which is afforded by the organic film deposited on its beam confronting surface, appears to continue, in some manner which is not as yet clearly understood, even after this organic film has been substantially evaporated by the bake-out operation, for screen structures manufactured in accordance with the process hereinbefore outlined show a greatly reduced tendency toward blemishes in the aluminum film even after extended periods of use following deposition of the indexing strips and incorporation of the screen into a completed cathode ray tube structure.

As has been pointed out, the deposition of indexing material on the aluminum film, as it was attempted unsuccessfully in the prior art, damaged the aluminum film either by reason of the direct impact of the particles of the indexing material or because some of this indexing material penetrated the aluminum film and caused swelling of the underlying film of organic material. When an organic protective film is interposed between the aluminum film and the indexing material in accordance with my invention, the latter becomes substantially incapable of causing damage in this manner. However, when the organic protective film is made, as it sometimes is, of such ingredients that it has very low viscosity, then small quantities of the most fluid ingredients of this protective film may penetrate through the intermolecular apertures in the aluminum film and may themselves cause sufficient swelling of the underlying supporting film to damage the aluminum film.

Where it is desired for any reason to use a protective organic film of such low viscosity, I have found that it is still possible to practice my invention to good advantage

provided certain additional precautions are also taken. The process which must be used in such a situation is illustrated diagrammatically in the flow chart of Figure 3, to which more particular reference may now be had. It will be apparent by inspection that the process illustrated in Figure 3 is similar to that illustrated in Figure 2 in its essential features. In particular, both processes are characterized by the application of a first organic film directly to colored light emissive phosphors of the screen structure and by the application of a second organic film to the aluminum film prior to the deposition of indexing material on the previously formed portions of the screen structure. However, the two processes differ in a number of important particulars. For example, the first step of the process illustrated in Figure 3, which is represented symbolically by rectangle 22, unlike the first step of the process of Figure 2, comprises not only the deposition of phosphor materials alone, but also the deposition of an inorganic binder material which is distributed more or less uniformly in the interstices between the phosphor particles in sufficient quantity to insure cohesion between these particles and adhesion thereof to the glass substrate. The next two steps of the method, respectively symbolized by rectangles 23 and 24 in Figure 3, are similar to the second and third steps (17 and 18) of Figure 2, consisting as did the latter, of the deposition of an organic film on the phosphors and of the deposition of an aluminum film on this organic film. But whereas, in the process of Figure 2, the second organic film was immediately applied to the aluminum layer, this is not done in the process of Figure 3. Instead, the previously formed portions of the screen structure, including the phosphor strips in their inorganic binder, the organic film and the aluminum film, are now dried and baked until the organic film is substantially completely vaporized. Only after this step, which is symbolically represented by rectangle 25 in Figure 3, is completed, is the second organic film deposited on top of the aluminum film. This last-mentioned step is symbolized by rectangle 26 of Figure 3. Thereafter indexing strips are deposited on the organic film, as symbolized by rectangle 27, and the resultant screen structure is dried and baked, as symbolized by rectangle 28, and is thus brought to completion in the same manner as in the process of Figure 2.

Thus it will be seen that the process of Figure 3 differs from that of Figure 2 principally in the addition of an inorganic binder material to the phosphor strips and in an additional drying and baking operation which is carried out after the deposition of the aluminum film and before the deposition of the second organic film thereon. The purpose of the additional drying and baking step 25 is to rid the screen structure of the first deposited organic film before the second organic film is applied. Once this has been done, it is clearly immaterial whether or not ingredients of the second inorganic film penetrate the aluminum layer for there is now no organic film present beneath this aluminum layer which could be swelled by this penetrating material. Consequently no damage to the aluminum film can be caused by such penetration. At the same time, however, the cohesive effect of the organic film, which is deposited prior to deposition of the aluminum film on the phosphors and which it is preferred to retain until the final bake-out of the tube, is also lost by the intermediate bake-out operation which vaporizes this organic film. The inorganic binder material, which is not susceptible to vaporization by this bake-out operation, is provided to substitute for the first organic film in this respect. Inorganic binders suitable for this purpose are potassium silicate and sodium silicate, but many others are, of course, also available.

In the foregoing discussion, my novel method has been described in its application to the deposition of secondary electron emissive indexing elements. However, it will be recalled that sometimes photoelectric indexing elements are preferred. It is therefore desired to emphasize that

## 11

by the practice of my novel method it is equally feasible to deposit light emissive phosphors on top of the aluminum film as it is to deposit secondary electron emissive materials, the essential requirement in either case being the aforementioned prior deposition of the intervening protective film.

It will be understood that other modifications of the manufacturing methods hereinbefore described in detail will occur to those skilled in the art without departing from my inventive concept. Accordingly I desire to limit the scope of this concept only by the appended claims.

I claim:

1. The method of depositing inorganic material on the surface of a film of metallic conductive material, said film being sufficiently thin to be permeable to the electrons of a cathode ray beam impinging thereon, said method comprising the steps of depositing a film of heat removable, film forming organic material on said conductive film, depositing said inorganic material on said organic film, and heating the structure so formed until said organic film is substantially completely vaporized.

2. The method of depositing particles of inorganic material on the surface of a metallic film, said metallic film being sufficiently thin to be permeable to the electrons of a cathode ray beam impinged thereon and said metallic film being suspended between spaced protrusions from a substrate, said method comprising the steps of depositing a film of heat removable, film forming organic material on said metallic film, depositing said particles of inorganic material on said organic film, and heating the structure so formed until said organic film is substantially completely vaporized.

3. The method of forming a screen structure for cathode ray tubes on a substrate of solid material, said method comprising the steps of: depositing a layer of phosphor materials on said substrate, depositing a first film of heat removable, film forming organic material on said phosphor layer, depositing a metallic film on said organic film, said metallic film being sufficiently thin to be permeable to the electrons of a cathode ray beam, depositing a second film of heat removable, film forming organic material on said metallic film, depositing on said second organic film a layer of material having a response characteristic to electron impingement which is substantially different from the response characteristic of said metallic film to electron impingement, and heating the structure so formed until both of said organic films have been substantially completely vaporized.

4. The method of forming a screen structure for cathode ray tubes on a substrate of solid transparent material, said method comprising the steps of: depositing a fluorescent screen on said substrate, depositing a first film of heat removable, film forming organic material on said fluorescent screen, depositing a metallic film on said first organic film, said metallic film being sufficiently thin to be permeable to the electrons of a cathode ray beam, depositing a second film of heat removable, film forming organic material on said metallic film, depositing on said second organic film material having a response characteristic to electron impingement which is substantially different from the response characteristic of said metallic film to electron impingement, said last-named material being deposited in predetermined geometrical configuration relative to said fluorescent screen, and heating the structure so formed until both of said organic films have been substantially completely vaporized.

5. The method of forming a screen structure for cathode ray tubes on a substrate of solid transparent material, said method comprising the steps of: depositing a fluorescent screen on said substrate, depositing on said fluorescent screen a film of heat removable, film forming organic material comprising a relatively low percentage of plasticizer, depositing a metallic film on said organic film, said metallic film being sufficiently thin to be permeable to the electrons of a cathode ray beam and sufficiently thick to

## 12

be substantially non-permeable to light emitted from said fluorescent screen, depositing on said metallic film a film of heat removable, film forming organic material comprising a relatively high percentage of plasticizer, depositing on said last-named organic film a layer of material having a response characteristic to electron beam impingement which is substantially different from the response characteristic of said metallic film to electron impingement, and heating the structure so formed until both of said organic films have been substantially completely vaporized.

6. The method of claim 5 further characterized in that said organic material constituting said second organic film comprises a sufficiently high percentage of plasticizer so that said second organic film will not contract appreciably during heating.

7. The method of forming a screen structure for cathode ray tubes on a substrate of solid transparent material, said method comprising the steps of: depositing on said substrate a layer of phosphor materials in an inorganic binder, depositing a first film of heat removable, film forming organic material on said phosphor layer, depositing a metallic film on said organic film, said metallic film being sufficiently thin to be permeable to the electrons of a cathode ray beam, heating the structure so formed until said first organic film is substantially completely vaporized, depositing a second film of heat removable, film forming organic material on said metallic film, depositing on said second organic film a layer of material having a response characteristic to electron impingement which is substantially different from the response characteristic of said metallic film, and heating the structure so formed until said second organic film is substantially completely vaporized.

8. The method of claim 4 further characterized in that said fluorescent screen comprises different portions constituted of phosphors emissive of light of different primary colors and disposed in a predetermined geometrical pattern.

9. The method of claim 4 further characterized in that said material deposited on said second organic film has a secondary electron emission ratio substantially greater than that of said metallic film.

10. The method of claim 9 further characterized in that said material of high secondary electron emission ratio is magnesium oxide.

11. The method of forming a screen structure for cathode ray tubes on a glass substrate, said method comprising the steps of: depositing a phosphor screen on said substrate, depositing a first film of organic material on said phosphor screen, depositing an aluminum film on said organic film, said aluminum film being sufficiently thin to be permeable to the electrons of a cathode ray beam, depositing a second film of organic material on said metallic film, said organic material of said second film being a composition of nitrocellulose, water insoluble plasticizer therefor, and octyl acetate dissolved in a volatile ester, depositing on said second organic film a layer of material having a response characteristic to electron impingement which is substantially different from the response characteristic of said aluminum film to electron impingement, and heating the structure so formed until both of said organic films have been substantially completely vaporized, the percentage of plasticizer in said composition constituting said second organic material being sufficiently high so that no substantial contraction of said second film of organic material takes place during said vaporization of organic films.

12. The method of forming a screen structure for cathode ray tubes on a substrate of solid material, said method comprising the steps of: depositing a layer of phosphor materials on said substrate, depositing a first film of heat removable, film forming organic material on said phosphor layer, depositing a metallic film approximately 1000 Angstrom units thick on said organic film,

**13**

depositing a second film of heat removable, film forming organic material on said metallic film, depositing on said second organic film a layer of material having a response characteristic to electron impingement which is substantially different from the response characteristic of said metallic film to electron impingement, and heating the structure so formed until both of said organic films have been substantially completely vaporized.

13. The method of forming a screen structure for cathode ray tubes on a substrate of solid material, said method comprising the steps of: depositing a layer of phosphor materials on said substrate, depositing a first film of heat removable, film forming organic material on said phosphor layer, depositing a metallic film on said organic film, said metallic film being sufficiently thin to be permeable to the electrons of a cathode ray beam, depositing a second film of heat removable, film forming organic material on said metallic film, spraying onto said second organic film particles of a material having a response characteristic to electron impingement which is substantially different from the response characteristic of said metallic film to electron impingement, and heating the structure so formed until both of said organic films have been substantially completely vaporized.

**14**

14. The method of claim 13 further characterized in that said spraying of material onto said second organic film is carried out under pressure which exceeds atmospheric pressure by approximately one-half pound per square inch.

References Cited in the file of this patent

**UNITED STATES PATENTS**

|           |          |                |
|-----------|----------|----------------|
| 2,006,166 | Hofmann  | June 25, 1935  |
| 2,031,603 | Holt     | Feb. 25, 1936  |
| 2,384,500 | Stoll    | Sept. 11, 1945 |
| 2,407,146 | Fagan    | Sept. 3, 1946  |
| 2,597,617 | Campbell | May 20, 1952   |
| 2,644,855 | Bradley  | July 7, 1953   |

**FOREIGN PATENTS**

|        |               |                |
|--------|---------------|----------------|
| 17,242 | Great Britain | Sept. 29, 1904 |
|--------|---------------|----------------|

**OTHER REFERENCES**

Chicago Club, "Official Digest of the Federation of Paint and Varnish Production Clubs" (1945), pp. 493-503.